

March 31, 1953

L. R. KOLLER

2,633,426

METHOD OF FORMING A POWDER COATING ON A SURFACE

Filed July 7, 1950



Inventor:  
Lewis R. Koller,  
by Paul A. Frank  
His Attorney.

## UNITED STATES PATENT OFFICE

2,633,426

METHOD OF FORMING A POWDER COATING  
ON A SURFACELewis R. Koller, Schenectady, N. Y., assignor to  
General Electric Company, a corporation of  
New York

Application July 7, 1950, Serial No. 172,449

15 Claims. (Cl. 117—27)

1

This invention relates to powder coatings and to methods of making such coatings. The present application is a continuation-in-part of application Serial No. 95,415, filed May 26, 1949, now abandoned, and assigned to the same assignee as the present application.

Heretofore, powder coatings have been produced by various methods. One process comprises forming a suspension of the powder to be coated in a suitable fluid vehicle and allowing the desired quantity of powder to settle under the influence of gravity on the coating supporting base. Such a process produces satisfactory coatings when only a gross, relatively porous coating of non-uniform and non-reproducible thickness, and which has a haphazard distribution of particles, is desired. This method does not lend itself to the manufacture of smooth coatings in which the powder particles are uniformly deposited in a layer of predetermined thickness.

Another prior art coating method comprises spraying a suspension of powder particles and binder on the base member to be coated. This method again produces a coating which is not easily controlled as to particle distribution and uniformity and magnitude of thickness. In still another representative prior art process a layer of binding material is applied to a base and the powder dusted or sprayed thereon. Inherent in this method are the same disadvantages discussed above whereby non-uniform, unreproducible coatings are obtained.

An object of this invention is to provide a powder coating of uniform and selected thickness.

Another object is to provide a method whereby powder coatings having a precisely controlled and uniform reproducible distribution of particles are produced.

Another object is to provide a method whereby powder coatings having monoparticle thick coating layers may be made.

A still further object of this invention is to provide a method of coating articles with powders wherein successive layers of uniform thickness and distribution of selected particles are obtained.

Other objects will become apparent from a consideration of the following description and

2

the drawing in which Fig. 1 is a perspective view of apparatus for carrying out the present invention; Fig. 2 is a perspective view of a plate having thereon a coating prepared according to the present process; Fig. 3 is a partial cross-sectional view of a coating produced by the process of this invention; and Fig. 4 is a perspective view of apparatus for coating irregular articles.

It has been found that superior powder coatings may be made by forming a layer of powder particles on the surface of a suitable liquid, transferring the layer to the surface to be coated, such as a glass plate or disc, and drying.

More particularly, it has been found that smooth and uniformly distributed reproducible powder coatings of controlled thickness may be quickly and easily produced by floating discrete liquid-repellent powder particles on a liquid medium to form a dispersed layer one particle thick compressing the particle layer to form a compact continuous film or layer one particle thick thereafter transferring the compacted layer to a surface desired to be coated, and drying.

The present invention may be applied to powdered materials in general, including both materials of inorganic, mineral, and organic origin, which are not deleteriously changed by contact with, or dissolved in, the liquid medium. Thus, powdered mica, titanium dioxide, silica, many powdered resins, and the like, may be used in the present application with water, and other liquid media. The invention is particularly applicable also to that class of materials known as phosphors which are used in making fluorescent screens such as those employed in television picture tubes and other apparatus where production of light by means of various exciting media is desired. Examples of such phosphors are zinc silicate, zinc sulfide, cadmium sulfide,

zinc-cadmium sulfide, magnesium silicate, cadmium borate, and beryllium silicate. Other examples of phosphors may be found in such works as "Introduction to Luminescence of Solids," H. W. Leverenz, Wiley, 1950, and "Some Aspects of the Luminescence of Solids," F. A. Kröger, Elsevier, 1948. Phosphor screens formed by the present process are smooth, of uniform thickness, and closely adherent to the base material. They are characterized by good definition, resolving

50 powder and contrast.

In the practice of this invention, it is necessary that the powdered materials to be coated be naturally repellent or rendered repellent to the liquid carrying medium on which they are floated to prevent their sinking in the medium. While various liquids may be chosen which will not wet certain specific powders, or conversely, powders chosen which will not be wet by a specific liquid, it is preferable to use water as a readily obtainable carrier medium and to treat the powders, if necessary, to make them water repellent. By this process, water may be used as the carrier medium for all powders desired to be coated. If the powder is one which is not wetted by water, it is, of course, not necessary to treat it with a water-repellent. If, however, the powder is one which is wetted by water, it may be treated with any of the well known water repellents, such as aluminum naphthenate, various stearates and other wax-like materials. Preferred for the water-repellent treatment in connection with the practice of this invention is the use of organo chlorosilanes, including those described in Patnode Patent 2,306,222, assigned to the same assignee as the present application. The specific repellent agent preferred is a mixture of methyl chlorosilanes comprising about thirty mol per cent dimethyl dichlorosilane and about seventy per cent methyl trichlorosilane. It has been found that 0.1% to 6% by weight of the organo silanes mentioned above added to powders will cause them to become water-repellent and to spread readily on a water surface. For the very best results from 1% to 4% by weight of the organo chlorosilane may be used. The treating agent may be added in any preferred manner to the powder which is kept in a state of agitation during addition or mixed after the material is added. Thus, the water-repellent material may be added drop-by-drop or in small increments or sprayed onto the powder or added in the form of a vapor. For small batches, the agent may be added to the powder in a jar, after which the jar is closed and shaken. The powder treated with silicon halide is spread out in a thin layer for several minutes in the air to allow the hydrogen halide formed to escape. The powder particles may also be made water-repellent by treating with silicone oil. Usually the silicone oil is used as a water emulsion in concentrations of up to about 5%. The amount of emulsion mixed with the powder ranges from about 0.01 to 0.04 per cent of the weight of the powder which is then oven dried, say at 90° C. to 150° C., or air dried. While several specific methods of waterproofing the powder are given herein, other well known methods, which are intended to be covered herein, will occur to those skilled in the art.

The powder, which is either inherently water-repellent or artificially so by reason of the above treatment, may be placed on the water in any convenient way. The water-repellent powder usually spreads readily over the surface of the water, even if deposited thereon in lumps. In some cases, it may be necessary to scatter the powder somewhat to cause it to spread. It is preferred to apply the powder by shaking through a screen or cloth, though an air blown spray, sprinkling or dusting or other well known methods will serve just as well. For a matter of a minute or so after the powder is deposited on the water surface, it undergoes a great deal of activity, during which time any aggregates

are broken down and a thin film of powder one particle deep is formed on the water surface. However, this film is so sparse or dispersed that the particles therein are relatively widely separated. In order, therefore, to obtain a continuous coating which is one particle deep or thick, it is necessary to compress the water film or coating, or reduce its area, after which a plate or other base material to be coated may be raised upward through the film from underneath the surface of the water, the film adhering to the surface of the plate.

For specific examples of the operation of the present process, reference is made to the drawing. By one method, as illustrated in Fig. 1, a receptacle such as shown at 1 is first filled with water 2 which is as free from foreign matter as possible. Preferably, the edges of receptacle 1 are coated with paraffin or similar waxy material, as shown at 3, so that the water level may be carried slightly above the receptacle edges. In order to remove any remaining traces of foreign matter such as dirt or grease from the surface of the water 2, a clean bar similar to barrier 4 is placed crosswise on the edges of the receptacle at one end and drawn over the entire water surface, its leading edge carrying away any foreign material. A clean water surface is necessary to insure uniform and constant behavior of the powder on the water surface. The powder to be coated, if not inherently water-repellent, is treated as disclosed above with a water-repellent agent. It is then deposited on the water surface by sifting through a screen, sprinkling, dusting, spraying, or by any other convenient method. Just enough powder is deposited to give a dispersed coating, such as that shown at 6. Up to several minutes are allowed for any aggregates of powder to break up and disperse over the liquid surface. The dispersed coating 6, so obtained, may be used as such if desired, but usually, as in the case of phosphor coatings for fluorescent screens, for example, it is desirable to have a continuous, uniform layer or coating of particles one particle thick or more. It is, therefore, necessary to compress or concentrate the dispersed coating into a compact aggregation, such as is shown at 6. This may be readily accomplished by drawing relatively together two barriers, such as bars 4 and 5, which rest on the edges of receptacle 1. By so moving the barriers toward one another, the concentration of powder particles per unit area of water surface is increased. If the particle concentration is so increased until incipient cracks or wrinkles begin to form, a continuous coating one particle deep, as at 7, is attained.

The thoroughly cleaned article or base material, such as glass slide 8 whose upper surface is to be coated, is next raised through the coating powder film 7 from beneath the water surface, the surface to be coated carrying away the film contacted by its area. The coating thus deposited may be dried by passing over it a gentle current of warm air. A holder such as that shown at 9 may be used to raise plate or slide 8 through film 7. As shown, this holder has a shank portion 10 to which are attached arms so shaped that they hold plate 8 without contacting its upper surface. These arms are also so bent that they pass under the barrier, such as 4, and permit the slide 8 to be raised vertically through the water surface and film 7 without displacing the barriers or otherwise breaking the film 7 before a portion of it has been deposited

on the upper surface of slide 8. While a particular design of holder has been described, it is to be understood that the holder may be shaped differently to accommodate discs, squares, and other variously shaped articles to be coated singly or together.

In actual practice, it has been found that as the wet film on a slide or other solid surface is dried, a slight compression of the coating occurs which tends to produce wrinkles. These objectionable wrinkles may be held to a minimum or obviated entirely by allowing the film on the water surface to expand slightly, say about one-tenth of its compressed area, after it has been compressed as described above. This is very easily accomplished by moving one or both of the barriers 4 or 5 toward its end of receptacle 1 the proper amount.

A slide having a coating deposited according to the above process has an appearance such as that presented in Fig. 2, the stippling representing a uniform coating 12 of dry particles one layer deep on slide 8, such as is shown in the magnified sectional view in Fig. 3. It will be noted from Fig. 3 that the particles 13 of powder in the coating are arranged uniformly with a minimum of discontinuity over the surface of the base material 8 in a layer one particle thick. The coatings of the present invention are of definite advantage when compared with coatings made by the above-mentioned prior art methods.

Monoparticle thick powder coatings may be also formed on a base material by passing the surface to be coated substantially vertically through the powder layer. During the process the powder layer on the liquid is subjected to a constant lateral pressure directed toward the surface to be coated to permit an even, continuous monoparticle coating to be applied to the base material as it is passed upward through the layer. Most of the water or liquid carried onto the base material along with the powder drains off from under the film as the base is elevated. This removal of water by draining from under the coating as the latter is placed on the base substantially reduces the time of drying over that when the surface to be coated is elevated through the liquid layer horizontally or parallel to the layer. By adjusting the lateral pressure on the powder layer as it is transferred from the liquid to the vertically rising surface so that the layer is in continuous contact with the base, irregular shaped surfaces, including those having both protruding and re-entrant surfaces, may be coated with a monoparticle layer of powdered material. Thus, corrugated surfaces, as concave, convex and other vari-shaped surfaces may be so coated.

For a specific example of the process of coating a non-planar surface, reference is made to Fig. 4. Receptacle 14, similar to receptacle 1 except that it is usually deeper to accommodate a vertically disposed base, is filled with water 15 as free as possible from foreign materials. Waxy material 16, such as paraffin and the like, is placed on the upper edges of the receptacle to allow the water level to be carried slightly above the receptacle edges. A barrier in the form of a clean metal bar may be drawn over the water surface to further remove any foreign material, such as dirt particles and the like. The powdered material to be deposited, which is treated with a water-repellent if it is not already water-repellent, is deposited on the water

surface, as described above, to provide a dispersed coating as at 17. The dispersed coating 17 is then compressed to a continuous monoparticle thick layer by drawing together two barriers 18 and 19 which are similar to 4 and 5. Again the presence of a continuous coating one particle thick 20 is denoted by the formation of incipient cracks or wrinkles in the layer surface. The thoroughly cleaned base material, such as the corrugated article 21, shown extending partly out of the liquid, whose front surface is to be uniformly coated, is next raised vertically upward through the powder layer surface by means of a holder such as that shown at 21. As the base 21 is slowly raised upward through layer 20, barrier 18 is moved toward barrier 19 to maintain a constant lateral pressure on the film 20 as it is pressed against 21 and to maintain the monoparticle thick nature of the layer on liquid 15 as it is transferred to coat 21. By maintaining a constant lateral pressure on layer 20 and, hence, an even pressure of layer 20 against the article 21 to be coated, a uniform monoparticle thick layer is deposited on 21 regardless of the shape of the latter. While 21 is shown in the figure as having a corrugated shape, it may be planar or of any irregular shape whatsoever.

As the article being coated rises above the surface of the water, the water or other liquid carried along with the coating material onto the article substantially completely drains off so that very little drying is necessary. Articles so coated take less time to dry than those made as in Fig. 1 in which case the moisture has to evaporate through the coating thickness. The final coating is similar to that shown in Fig. 3 except that the base need not be planar.

Any number of successive coatings may be formed by the method illustrated in Fig. 4 so long as each coating is dried before the succeeding one is applied.

Powder coatings made according to the present process adhere to the material coated without the aid of adhesives and will resist usual handling or jarring so long as the coating itself is not brushed or scraped. If it is desired to add additional layers of the same or a different powder to the base layer, it is best to thoroughly air dry or heat dry the screen or slide with the first layer to waterproof the coating. Once the previously coated layer has been thus treated, it may be immersed in water without danger of stripping. Any number of layers may be added successively so long as each previous layer is dried as above.

What I claim as new and desire to secure by Letters Patent of the United States is:

1. The method of forming a powder coating one particle thick on a surface which comprises rendering the powder particles liquid-repellent, floating said powder particles on a clean liquid surface to form a dispersed powder layer thereon, reducing the area of the powder layer until the appearance of incipient wrinkles in the layer, passing the surface desired to be coated upward through the powder layer and thereafter drying the coating.

2. The method of forming a powder coating on a surface which comprises rendering powder particles water-repellent, floating the powder particles on water to form a powder layer, compressing the area of the powder layer until the appearance of incipient wrinkles in the layer, releasing the compression to allow about a one-

tenth increase in the compressed area, passing the surface desired to be coated upward through the powder layer and drying the coated surface.

3. The method of forming successive coatings one particle thick on a surface which comprises floating liquid-repellent powder particles on a clean liquid surface to form a dispersed powder layer thereon, reducing the area of the powder layer until the appearance of incipient wrinkles in the layer, enlarging the reduced area about one-tenth, passing the surface to be coated upward through the powder layer, drying the coating and repeating the coating process.

4. The method of forming a fluorescent screen coating comprising successive layers of phosphor material which comprises floating liquid-repellent phosphor powder particles on a liquid carrier medium to form a powder layer, compressing the area of the powder layer until the appearance of incipient wrinkles or cracks in the layer, enlarging the compressed area about one-tenth, passing the surface to be coated upward through the powder layer, drying the coating and repeating the process as desired.

5. The method of forming a powder coating on an irregularly shaped base member which comprises floating liquid-repellent powder particles on a liquid carrier medium to form a powder layer, compressing the powder layer laterally to form a compact aggregation of powder particles and thereafter transferring the compacted layer to the base member by passing the surface substantially vertically upward through the powder layer while maintaining a constant lateral pressure on the powder layer directed toward the surface to be coated.

6. The method of forming a powder coating on an irregularly shaped base member which comprises treating discrete powder particles with a liquid-repellent agent, floating the treated particles on a liquid carrier medium to form a powder layer, exerting lateral compression on the floating powder layer to form it into a compact aggregation and thereafter transferring the compacted layer to the surface desired to be coated by passing the surface substantially vertically upward through the powder layer while maintaining a constant lateral pressure on the powder layer directed toward the surface to be coated.

7. The method of forming a fluorescent screen one particle thick on an irregularly shaped base member which comprises floating liquid-repellent powder particles on a liquid carrier medium to form a powder layer, compressing the area of the powder layer until the appearance of incipient wrinkles therein, allowing the compressed powder layer to expand about one-tenth of its compressed area, and thereafter transferring the powder layer to the base member by passing the surface substantially vertically upward through the powder layer while maintaining a constant lateral pressure on the powder layer directed toward the surface to be coated.

8. The method of forming a powder coating on a surface which comprises rendering powder particles water-repellent by treating the particles with a material selected from the class consisting of silicone oil and organo chlorosilane, floating the powder particles on water to form a powder layer thereon, compressing the area of the powder layer until the appearance of incipient wrinkles in the layer, passing the surface to be coated upward through the powder layer and drying the coated surface.

9. The method of forming a powder coating on

a surface which comprises rendering powder particles water-repellent by treating the powder particles with an organo chlorosilane, floating the powder particles on water to form a powder layer thereon, compressing the area of the powder layer until the appearance of incipient wrinkles in the layer, releasing the compression to allow about a one-tenth increase in the compressed area, passing the surface desired to be coated upward through the powder layer and drying the coated surface.

10. The method of forming a powder coating on a surface which comprises rendering powder particles water-repellent by treating the powder particles with a methyl chlorosilane, floating the powder particles on water to form a powder layer thereon, compressing the area of the powder layer until the appearance of incipient wrinkles in the layer, releasing the compression to allow about a one-tenth increase in the compressed area, passing the surface desired to be coated upward through the powder layer and drying the coated surface.

11. The method of forming a powder coating on a surface which comprises rendering powder particles water-repellent by treating the powder particles with a mixture of methyl chlorosilanes comprising about 30 mol per cent dimethyl chlorosilane and about 70 per cent methyl trichlorosilane, floating the powder particles on water to form a powder layer thereon, compressing the area of the powder layer until the appearance of incipient wrinkles in the layer, releasing the compression to allow about a one-tenth increase in the compressed area, passing the surface desired to be coated upward through the powder layer and drying the coated surface.

12. The method of forming a fluorescent screen on an irregularly shaped base member which comprises floating liquid-repellent phosphor powder particles on a liquid carrier medium to form a powder layer, compressing the powder layer until the appearance of incipient wrinkles in the layer, and thereafter transferring the compacted layer to the base member by passing the surface substantially vertically upward through the powder layer while maintaining a constant lateral pressure on the powder layer directed toward the surface to be coated.

13. The method of forming a powder coating on a surface which comprises rendering the powder particles water-repellent by treating the powder particles with a mixture of methyl chlorosilanes comprising about 30 mol per cent dimethyl dichlorosilane and about 70 mol per cent methyl trichlorosilane in the amount of 0.1 per cent to 6 per cent by weight based on the weight of the powder particles, floating the powder particles on water to form a powder layer thereon, compressing the area of the powder layer until the appearance of incipient wrinkles in the layer, releasing the compression to allow about a one-tenth increase in the compressed area, passing the surface desired to be coated upward through the powder layer and drying the coated surface.

14. The method of forming a powder coating on a surface which comprises rendering powder particles water-repellent by treating the particles with a silicone oil, floating the particles on water to form a powder layer thereon, compressing the area of the powder layer until the appearance of incipient wrinkles therein, passing the surface to be coated upward through the powder layer and drying the coated surface.

15. The method of forming successive powder

coatings one particle thick on a surface which comprises rendering the particles water-repellent by treating with a material selected from the group consisting of silicone oil and organo chlorosilane, floating the particles on water to form a powder layer thereon, compressing the area of the powder layer until the appearance of incipient wrinkles therein, passing the surface to be coated upward through the powder layer and drying the coated surface.

LEWIS R. KOLLER.

## REFERENCES CITED

The following references are of record in the file of this patent:

## UNITED STATES PATENTS

|    | Number    | Name            | Date           |
|----|-----------|-----------------|----------------|
| 5  | 304,802   | Dewar           | Sept. 9, 1884  |
|    | 2,220,860 | Blodgett        | Nov. 5, 1940   |
|    | 2,278,742 | Scott et al.    | Apr. 7, 1942   |
| 10 | 2,385,615 | Dreyer          | Sept. 25, 1945 |
|    | 2,424,853 | Safford         | July 29, 1947  |
|    | 2,493,745 | Blodgett et al. | Jan. 10, 1950  |